

# UNITED STATES PATENT OFFICE.

EMIL L. MANHAYFER, OF ST. LOUIS, MISSOURI.

## TOUGHENED-PITCH COMPOSITION.

1,112,817.

Specification of Letters Patent.

Patented Oct. 6, 1914.

No Drawing.

Application filed December 13, 1910. Serial No. 597,163.

To all whom it may concern:

Be it known that I, EMIL L. MANHAYFER, a citizen of the United States, and resident of St. Louis, Missouri, have invented certain new and useful Improvements in Toughened-Pitch Compositions, of which the following is a specification.

This invention relates to a composition of matter for roofing, paving and flooring purposes. The same is accomplished by first reducing the pitch to a liquid state, thoroughly agitating the same, and during the process of agitation by applying and mixing the pitch with infusorial earth or kieselguhr of such quantity and proportion as to cause the pitch, after it has been placed in containers to assume a plastic toughened state.

Heretofore it has been proposed to saturate and cover both sides of a woven or textile fabric or felt cloth with coal tar in which there has been incorporated sufficient infusorial or diatomaceous earth to produce a cement capable of rendering cloth or the like practically fire-proof, for example, it has been proposed to employ 25 parts of infusorial earth and 75 parts of coal tar, the same being thoroughly mixed together and heated to bring the same to a fluid consistency. The fabric was then drawn through this fluid bath and the excess of the liquid composition forced out of the fabric by pressure rollers. The cloth thus treated was then passed through a so-called dust bath composed of pulverulent infusorial earth, with the result that the same adhered to the treated cloth, and the product was then hung up. As soon as the infusorial dust thus applied had absorbed all the liquid tar that it was capable of, the dust bath was repeated a sufficient number of times to accomplish the necessary absorption of the liquid tar. Usually two applications of the dust bath sufficed. After the cloth had been finished in the manner aforesaid, in order to prepare the same for market it was made up into rolls and during the process of rolling it was sifted with a powder absorbing material, such as diatomaceous earth, soap-stone, or other suitable material, to prevent the layers from sticking together.

The foregoing cementitious material is not suitable as a substitute for material produced by the process herein described, and

such process as described is accordingly disclaimed by me as being intended to be included within the scope of the claims annexed to this specification or hereinafter inserted therein.

What I do claim and desire to secure by Letters Patent is, the treatment of pitch, which is a product distinctly different from tar, and which has a recognized and distinct technical status. Pitch is a residual product of tar being defined as (see *Standard Dictionary*, Funk & Wagnalls, 1909):—“a thick, dense, black or dark-brown substance obtained by boiling down tar and from the residues of distilled turpentine.”

In carrying out my invention I preferably proceed as follows:—A mass of pitch, by which term is included the residue of tars and oils, such as coal-tar pitch, oil-tar pitch, pine-tar pitch, candle-tar pitch, asphalt and the like, is first reduced to a liquid state and thoroughly agitated while simultaneously adding sufficient infusorial earth or kieselguhr in such proportion as to cause said pitch after it had been removed and placed in containers and allowed to cool, to assume a plastic toughened state, in which condition it is sufficiently hard to be capable of withstanding the natural heat of the sun's rays, for example, it will possess a melting point approximately 200° F. and yet be sufficiently tough and adhesive to retain the gravel partially embedded therein under varying conditions of service. As a result of the incorporation of said kieselguhr therewith, the said resultant product will be prevented from “running” under the natural heat of the sun as is the case with ordinary pitches when placed on sloping roofs or inclined surfaces, and also the pitch is rendered more fire-proof and has ample adhesive quality. It is moreover sufficiently elastic to permit of expansion and contraction without cracking or breaking when subjected repeatedly to heat or cold.

When the requisite amount of kieselguhr in accordance with the above requirement is added to coal tar pitch, an amount for example from 15 to 20% is amply sufficient, the melting point of the same which would ordinarily be about 140° F. will be elevated to approximately 200° F., yet at the same time substantially all of the elasticity and

adhesiveness of ordinary pitch possessing a low melting point will be preserved. This intermingling of kieselguhr with the ordinary pitches results in the absorption and 5 retention of the liquid portions, such as any of the light oils, or other tar oils including heavy green oils thereof remaining unvapORIZED during the distillation process in the manufacture of such pitches. In addition 10 to this the kieselguhr *i. e.* infusorial earth, appears to act as an insulator against heat and cold. As a result of this absorption of the light oils, the finished product is apparently incapable of ultimately setting to a 15 brittle mass, as is customary with untreated pitches, with the result that the mass is permanently maintained in a plastic state and cracking or running due to cold or heat, is prevented as aforesaid.

20 The effect of the kieselguhr upon the pitch appears to be due partly to a chemical transformation which may be best explained on the theory, that partial oxidation of the anthracene to anthroquinone occurs, since 25 the melting point of the former is about 210° C. and the latter about 280° C. Apparently the kieselguhr in such a case serves as a catalytic agent during said agitation and heating of the melted pitch results in 30 the rapid oxidation of the same and consequent elevation of the melting point. Upon analysis for example, of untreated pitch an amount approximately 7% of crude anthracene was obtained, whereas upon analysis of 35 the fraction obtained from the dried pitch an amount up to 11% of crude anthroquinone containing traces of naphthalene possibly naphthaquinone was found.

The treatment of coal tar as distinguished 40 from coal tar pitch in the identical manner as above described, does not produce a combination which can satisfactorily be employed as a substitute for the product produced by applicant, for the reason that coal tar which is recognized as being an entirely distinct article commercially from 45 coal tar pitch, contains too large a proportion of light oils to permit of the necessary absorption of the same by a reasonable portion of kieselguhr. The only way in 50 which these oils can be taken care of is by some such process as that herein referred to as known in the prior art. This however is entirely unsatisfactory and has never been 55 commercially employed because of its impracticability. In fact it is impossible whether employing applicant's invention or the process herein described as known to the prior art, to directly add kieselguhr to 60 coal tar, as such, and obtain a product which has a high melting point and a low freezing point, and which is sufficiently resistant to the change in temperature, and sufficiently tough and elastic to permit of 65 walking thereon without damaging effect

due to puncturing of the layers thereof, and possess the other desirable properties herein described to a sufficient degree to render the same suitable for roofing and like purposes. It is obvious that any pitch containing 70 kieselguhr whether the same is obtained by direct addition of the kieselguhr to the pitch or by addition to the tars during distillation thereof from which pitch is produced, is equally within the scope of my invention, 75 but I distinctly disclaim on the other hand an end product consisting of undistilled tar which as is well known is permanently in a liquid condition, having incorporated therein a small or large amount of kieselguhr or 80 like material. It is obvious that since the direct heat of the sun's rays being in many cases approximately 150° F. that the increase in the melting point of this treatment will be at least in substantial excess of the 85 normal melting point of pitch of 140° F.

The essential feature of my invention is the intermingling of infusorial earth or kieselguhr with pitch in such quantities and proportions as to render the finished product 90 plastic.

By the word pitch referred to in the above is meant the residue of tars and oils, such as coal tar pitch, oil tar pitch, pine tar pitch, 95 cannel tar pitch, asphalt pitch and the like.

As kaolin, clay and like inert relatively heavy inorganic silicious substances are incapable of substitution for the inert absorptive materials of lower specific gravity which are capable of remaining substantially in permanent suspension in pitch herein referred to the same are hereby specifically disclaimed as being without the scope and spirit of my invention as embodied in 100 the accompanying claims.

Kieselguhr or infusorial earth is essentially different from kaolin, clay and like relatively heavy inorganic fillers and therefore its effect upon pitch is likewise quite dissimilar from such heavy fillers.

The following tabulated properties serve to emphasize the essential differences between infusorial earth or kieselguhr and such heavy fillers as clay, kaolin and the like, both alone and mixed with commercial pitch, (Table 1) giving the absorption, loose weight and specific gravity of the materials themselves;—and (Table 2) giving the melting point, slide and settling values of mixtures of kaolin-pitch and kieselguhr-pitch, 115 respectively.

Table 1.

|                       | Absorption<br>of cresylic<br>acid per<br>gram. | Loose<br>weight per<br>cubic foot. | Specific<br>gravity. | 125 |
|-----------------------|------------------------------------------------|------------------------------------|----------------------|-----|
| Infusorial earth..... | c. c.<br>1.9                                   | Lbs.<br>13.78                      | 1.69                 |     |
| Kaolin.....           | 0.5                                            | 65.06                              | 2.54                 |     |
| Pottery clay.....     | 0.2                                            | 61.94                              | 2.55                 | 130 |

Table 2.

| Pitch No. | Composition:               | Melting point, in air degrees F. | Slide in inches 7 hrs. @ 40° C. | Settling tests 4 hrs. @ 85°-90° C. Per cent. ash— |        |
|-----------|----------------------------|----------------------------------|---------------------------------|---------------------------------------------------|--------|
|           |                            |                                  |                                 | Before.                                           | After. |
| 5         | 15% kaolin                 | 128                              | 2.88                            | 12.92                                             | 9.89   |
|           | 15% infusorial earth       | 159                              | 0.50                            | 13.71                                             |        |
| 10        | Straight commercial pitch. | 125                              | 3.88                            | 13.69                                             |        |

It is evident from the foregoing that whereas infusorial earth or kaolin changes the properties of commercial pitch to a very considerable extent, when incorporated therewith in relatively small proportions, (for example 15%), to wit, the melting point is increased from 126° F. to 159° F. and the slide is decreased from 3.88" to less than 1 inch, and there is practically no settling of said kieselguhr even after four hours. On the other hand, kaolin in similar amounts has no material effect whatsoever upon the properties of the pitch, the melting point being changed not over 3° and the slide being decreased but a few per cent., to wit, about 25% as distinguished from over 85% in the case of kieselguhr and the settling being over 33% as distinguished from practically *nil* in the case of kieselguhr. Likewise as fully set forth in Table 1 the absorptive properties, loose weight and specific gravities of kieselguhr and kaolin are materially different.

Having thus fully described my invention, what I claim as new and desire to have secured to me by the grant of Letters Patent, is:

1. A composition of matter consisting of pitch having sufficient infusorial earth homogeneously incorporated therein to maintain the same plastic at normal temperatures and to increase the melting point thereof substantially in excess of the melting point of untreated pitch of a similar nature to the pitch therein contained.

2. A composition of matter consisting of pitch having sufficient kieselguhr homogeneously incorporated therein to render the same plastic at normal temperatures and to increase the melting point thereof substantially in excess of the melting point of untreated pitch of a similar nature to the pitch therein contained, and sufficient to resist, after the initial hardening of the same, the natural heat of the sun's rays without melting.

3. A composition of matter consisting of pitch having sufficient quantities of inert absorptive material homogeneously incorporated therewith to maintain the same plastic throughout a materially increased range of temperature, and to increase the melting

point thereof substantially in excess of the melting point of untreated pitch of a similar nature to the pitch therein contained, said inert absorptive material being characterized by a specific gravity not exceeding 2.00, an absorptive property of at least 1 cc. of cresylic acid per gram, a loose weight not exceeding 25 lbs. per cubic foot, being capable of increasing the melting point of ordinary pitch when incorporated therewith in amounts of 15% by at least 20° F., and being capable of remaining in suspension in said pitch without more than 15% settling at 85° to 90° C. during an interval of four hours.

4. A composition of matter consisting of pitch having sufficient quantities of inert absorptive material homogeneously incorporated therewith to maintain the same plastic throughout a materially increased range of temperature, and to increase the melting point thereof substantially in excess of the melting point of untreated pitch of a similar nature to the pitch therein contained, said inert absorptive material being characterized by a specific gravity not exceeding 1.8, an absorptive property of at least 1.5 cc. of cresylic acid per gram, a loose weight not exceeding 45 lbs. per cubic foot, being capable of increasing the melting point of ordinary pitch when incorporated therewith in amounts of 15% by at least 25° F. and being capable of remaining in suspension in said pitch without more than 10% settling at 85° to 90° C. during an interval of four hours.

5. A composition of matter consisting of pitch having sufficient quantities of inert absorptive material homogeneously incorporated therewith to maintain the same plastic throughout a materially increased range of temperature, and to increase the melting point thereof substantially in excess of the melting point of untreated pitch of a similar nature to the pitch therein contained, said inert absorptive material being characterized by a specific gravity exceeding 1.0 and not exceeding 1.8, an absorptive property of at least 1 cc. of cresylic acid per gram, a loose weight not exceeding 25 lbs. per cubic foot, being capable of increasing the melting point of ordinary pitch when incorporated therewith in amounts of 15% by at least 20° F. and being capable of remaining in suspension in said pitch without more than 15% settling at 85° to 90° C. during an interval of four hours.

In testimony whereof, I have signed my name to this specification, in presence of two subscribing witnesses.

EMIL L. MANHAYFER.

Witnesses:

ALFRED A. ERICO,  
WALTER C. STEIN.